

## UNITED STATES PATENT OFFICE

2,646,369

## PROCESS OF TRANSPARENTIZING PAPER

Robert R. Parmentier, Upper Darby, Pa.

No Drawing. Original application April 12, 1950,  
Serial No. 155,565. Divided and this applica-  
tion October 18, 1950, Serial No. 190,883

8 Claims. (Cl. 117—92)

1

This invention relates to compositions and processes for transparentizing fibrous materials such as paper.

It is often desired to reproduce copies of drawings, printed pages, or other similar materials. This may be accomplished by photographing the drawing and preparing prints from the so-obtained negative. A further method is to prepare prints directly from such page or drawing. In this latter method, the paper in general use is too opaque to permit the preparation of satisfactory prints, and in the photographic process the cost of the reproduction makes the process prohibitive in many instances. In order to overcome these and other difficulties, it has heretofore been suggested to employ various compositions in order to transparentize the paper from which reproductions are desired, and thus render the attainment of prints directly therefrom feasible. Compositions heretofore proposed, however, have serious disadvantages which greatly restrict or prevent their use. For example, compositions heretofore proposed suffer one or more of the following difficulties: the compositions may be dangerous to compound and use, are difficult to prepare and apply to the paper, drying thereof is slow, the material used in transparentizing, usually an oil, is transferred to prints and other papers which it contacts thus restricting its use and making storage of the treated paper difficult, odor is imparted to the treated paper which makes its use obnoxious and which permeates other papers and materials such as when stored together, tacking, i. e., sticking of the treated paper to hot surfaces of reproducing machines, which prevents or greatly limits their use in most processes, and lack of good transparentizing thus preventing the attainment of suitable reproductions.

An object of the present invention is to provide compositions effective to transparentize paper and obviate the above-mentioned difficulties. A further object is to provide a process for transparentizing papers.

The present invention comprises a novel transparentizing solution and its application to paper, preferably followed by application of a novel sealing solution, as hereinafter fully described.

The transparentizing solution of the present invention comprises mineral oil, 10-35 vol. %; toluene, 4-10 vol. %; and carbon tetrachloride, 55-80 vol. %. This composition is applied directly to the paper to be transparentized, preferably to the side thereof which does not contain the printed matter or drawing the reproduction

2

of which is desired. Application is conveniently accomplished by rubbing the paper with a cloth or sponge saturated with the transparentizing solution. Other means of application may be employed, such as spraying, brushing, and dipping. The composition of the present invention dries in a very short time, within about 2-5 minutes, and the so-treated paper may then be used in preparing photographic reproductions. It is preferred, however, to further treat the paper with a novel composition comprising wax, 2-6 vol. %; a gasoline hydrocarbon fraction, 31-47 vol. %; and carbon tetrachloride, 47-67 vol. %. This composition is described and claimed in my copending application, Serial Number 190,882, filed October 18, 1950. Using the stated ranges of gasoline and carbon tetrachloride, a saturated solution of the wax, at about room temperature, may advantageously be employed. It has been found that this composition effectively seals the paper so that no seepage is apparent even after long storage, and also provides other advantages as hereinafter described. The sealing composition may be applied in the same manner as described for the transparentizing composition.

In transparentizing paper in accordance with the present invention, the transparentizing solution may be applied to the paper and after drying the sealing solution applied. It is preferred to apply the sealing composition before the transparentizing solution is completely dry. It has been found that operating in this manner the total time of application of the solutions is considerably decreased, the sealing solution is more readily applied, and total drying time is decreased.

In the above-described transparentizing composition, it is possible to substitute xylene, usually as a mixture of the various xylenes, or benzene, in whole or in part, for the toluene. The oil employed is preferably a refined white mineral oil boiling in the lubricating oil range. The wax employed in the sealing solution is preferably a paraffin wax of petroleum origin having a melting point of from about 115° F. to 200° F., although microcrystalline wax of the same melting point range may be employed. Also, in place of the gasoline petroleum fraction there may be substituted one or more aliphatic hydrocarbons boiling within this range, such as normal and branched chain hexanes, heptanes, and octanes. Preferably there is employed a straight run de-aromatized gasoline fraction boiling within the range of from about 185° F. to 400° F.

It is important that the stated concentration ranges for the ingredients of both compositions be observed. With respect to the transparentizing composition, if mineral oil be employed in less than the stated amount, the paper is not sufficiently transparentized to permit satisfactory reproduction, whereas if more than the stated quantity is employed, the paper will be slow drying and seepage occurs; if less than the stated amount of toluene is employed seepage is observed, whereas if more than the stated quantity is employed the composition may be inflammable and has an offensive odor; if carbon tetrachloride is employed in less than the stated quantity, penetration of the paper by the transparentizing composition is decreased thereby making the application of the composition difficult, and the composition may be inflammable, whereas employing more than the stated quantity results in too fast drying which makes its application to paper difficult and uneven. With respect to the sealing composition, if less than the stated quantity of wax is employed, effective sealing will not be obtained so that seepage is observed, whereas if more than the stated quantity is employed, tacking during the reproduction operation is observed; if less than the stated quantity of gasoline is employed the wax will not be sufficiently soluble in the composition to achieve the desired results, whereas more than the stated quantity may render the composition inflammable; the same disadvantages of employing a quantity of carbon tetrachloride outside of the stated range is observed with sealing composition as with the transparentizing composition.

Various papers may be treated in accordance with the present process, and the so-treated papers used in various reproduction processes. Papers which may be treated for example include the usual bond paper of say about 13 to 24 lb. weight per 1000 sheets, photographic, tracing, chart, and blue print papers, and in general any paper except very heavy fibrous materials such as cardboard. The treated papers may be employed for making reproductions in a variety of processes involving the transmission of light through the treated paper. As illustrative of such processes may be mentioned direct printing such as contact box printing, the use of Ozalid, Bruning, blue print machines, and actinic light contact printing. The treated papers may also be used in projection printing.

The following examples illustrate preferred

and of the necessity of using the described ingredients in the present compositions, a series of solutions was prepared and tested. The compositions prepared were as follows (parts given as parts by volume):

Composition 1:

|            |   |
|------------|---|
| Castor oil | 1 |
| Turpentine | 1 |

Composition 2:

|                    |   |
|--------------------|---|
| Cocoanut oil       | 1 |
| Light paraffin oil | 1 |
| Benzine            | 1 |
| CCl <sub>4</sub>   | 1 |

Composition 3:

|                    |   |
|--------------------|---|
| Light paraffin oil | 1 |
| Benzine            | 1 |
| CCl <sub>4</sub>   | 1 |

Composition 4:

|                   |    |
|-------------------|----|
| Light mineral oil | 6  |
| Benzine           | 1  |
| CCl <sub>4</sub>  | 13 |

Composition 5:

|                                 |    |
|---------------------------------|----|
| Light refined white mineral oil | 6  |
| Toluene                         | 1  |
| CCl <sub>4</sub>                | 13 |

Composition 6:

|                                |    |
|--------------------------------|----|
| Straight run gasoline fraction | 8  |
| Wax                            | 1  |
| CCl <sub>4</sub>               | 12 |

It will be noted that Compositions 5 and 6 are the present transparentizer and sealing compositions, respectively. In Composition 6, the gasoline fraction employed was a straight run fraction boiling between about 190° F. and 380° F., and the wax employed was a paraffin wax having a melting point of 150° F. (A. S. T. M. D-87-42 method). Data obtained are presented in the following table, which gives the following data: (1) application, which is the ease of application of the composition to the paper—a measure of the rubbing and time required to apply the composition; (2) drying, which is the time required for the treated paper to dry; (3) odor, which is the odor of the treated paper after standing 6 days; (4) seepage, which is the tendency of the oil to rise to the surface of the paper, observed by transfer of oil from the treated paper to a contacting paper on standing 24 hours; and (5) transparency of the product, i. e., whether sufficient light will be transmitted through the paper to obtain good contact photoprints.

| Composition      | Application    | Drying <sup>1</sup> | Odor        | Seepage      | Transparency |
|------------------|----------------|---------------------|-------------|--------------|--------------|
| 1                | very difficult | very slow           | strong      | serious      | good.        |
| 2                | difficult      | slow                | do          | very serious | fair.        |
| 3                | moderate       | moderate            | do          | do           | poor.        |
| 4                | do             | slow                | do          | moderate     | fair.        |
| 5                | easy           | fast                | very slight | very slight  | good.        |
| 6                | do             | do                  | do          | none         | fair.        |
| 5+6 <sup>2</sup> | do             | do                  | none        | do           | good.        |
| 5+6 <sup>3</sup> | very easy      | do                  | do          | do           | Do.          |

<sup>1</sup> Drying times were as follows: Very slow=60+ minutes; slow=20-60 minutes; moderate=5-20 minutes; fast=2-5 minutes.

<sup>2</sup> Paper treated with composition 5 followed in 10 minutes (after drying) by treatment with composition 6.

<sup>3</sup> Paper treated with composition 5 followed immediately (before drying) by treatment with composition 6.

embodiments of the present invention and the superiority of the present compositions and processes over those heretofore known:

*Example 1*

In order to demonstrate superiority of the present compositions over those heretofore described,

As noted above, Composition 5 is the transparentizer and Composition 6 the sealer of the present invention. It is apparent that Composition 6 acts to transparentize paper, but gives only a fair product. The last two lines of the table represent preferred processes of the present invention, and show the excellent results achieved.

*Example 2*

In order to illustrate a preferred embodiment of the present process, it was desired to reproduce copies of an engineering drawing of size 30 by 41 inches, the size of the desired copies being 11 by 15½. The original drawing was photographed and a print of the desired size made on an opaque photographic paper from the negative. This print was transparentized and sealed using the compositions of the present invention as described, applying the sealing composition after drying of the transparentizing composition. The transparentized photo-print was then employed in an Ozalid machine to produce the desired number of prints, excellent results being achieved.

*Example 3*

It was desired to produce copies of a type-written report. The papers were transparentized and sealed in accordance with the present process and copies made directly therefrom on an Ozalid machine.

Untreated paper was tested against the transparentized paper and it was found that the speed of the machine using transparentized paper was increased from 2 to 4 times, and that the prints were sharper and contained greater contrast than those obtained with the untreated paper.

*Example 4*

Composition 5 of Example 1 was duplicated except that benzene was substituted for toluene. A blue-print of an engineering drawing was transparentized therewith and sealed with Composition 6 as described for Example 1. Substantially identical results were obtained as with toluene.

*Example 5*

Example 4 was repeated using a mixture of xylenes in place of toluene. Results substantially identical to those obtained in Example 4 were obtained.

*Example 6*

Six commercial transparentizers were purchased and results obtained therewith compared to those obtained with the compositions of the present invention. Each of the commercial compositions were slow drying, imparted a permanent odor to the paper, and exhibited serious seepage. The transparentizing ingredient of these compositions were vegetable oils, such as linseed or cocoanut oil.

This application is a division of patent application Serial No. 155,565, filed April 12, 1950 now Patent 2,616,815.

The invention claimed is:

1. Process for transparentizing paper which comprises applying a solution consisting of 10-35 vol.% mineral oil boiling in the lubricating oil

range, from 4-10 vol.% of a material selected from the group consisting of benzene, toluene, and xylene, and from 55-80 vol.% carbon tetrachloride to paper and then applying a sealing solution consisting of from 2-6 vol.% petroleum wax having a melting point of from 115° F. to 200° F., from 31-47 vol.% gasoline hydrocarbon fraction, and from 47-67 vol.% carbon tetrachloride to said paper.

10 2. Process according to claim 1 wherein toluene is the material selected from the group consisting of benzene, toluene, and xylene.

15 3. Process of transparentizing paper which comprises applying to paper a transparentizing solution consisting of 10-35 vol.% mineral oil boiling in the lubricating oil range, from 4-10 vol.% toluene, and from 55-80 vol.% carbon tetrachloride, drying the treated paper, and applying a sealing composition consisting of 2-6 vol.% petroleum wax having a melting point of from 115° F. to 200° F., from 31-47 vol.% of a gasoline hydrocarbon fraction, and from 47-67 vol.% carbon tetrachloride.

20 4. Process of transparentizing paper which comprises applying to paper a transparentizing solution consisting of 10-35 vol.% mineral oil boiling in the lubricating oil range, from 4-10 vol.% toluene, and from 55-80 vol.% carbon tetrachloride, and subsequently applying before drying of said transparentizing solution a sealing composition consisting of 2-6 vol.% petroleum wax having a melting point of from 115° F. to 200° F., from 31-47 vol.% of a gasoline hydrocarbon fraction, and from 47-67 vol.% carbon tetrachloride.

25 5. Process according to claim 1 wherein benzene is the material selected from the group consisting of benzene, toluene, and xylene.

30 6. Process according to claim 1 wherein xylene is the material selected from the group consisting of benzene, toluene, and xylene.

35 7. Process for transparentizing paper which comprises applying a solution consisting of 10-35 vol.% mineral oil boiling in the lubricating oil range, from 4-10 vol.% of a material selected from the group consisting of benzene, toluene, and xylene, and from 55-80 vol.% carbon tetrachloride to paper and then applying a sealing solution consisting of from 2-6 vol.% petroleum wax having a melting point of from 115° F. to 200° F., from 31-47 vol.% of an aliphatic hydrocarbon boiling within the gasoline range, and from 47-67 vol.% carbon tetrachloride to said paper.

40 8. Process according to claim 1 wherein said gasoline hydrocarbon fraction is a straight run dearomatized gasoline hydrocarbon fraction.

ROBERT R. PARMENTIER.

No references cited.